

May 9, 1961

C. A. STEPHENS ET AL

2,983,131

MANUFACTURE OF COATED LEATHER SHAFT SEALS

Original Filed Oct. 12, 1955



FIG. 1



FIG. 2



FIG. 6



FIG. 3



FIG. 4



FIG. 5

## 1

2,983,131

MANUFACTURE OF COATED LEATHER  
SHAFT SEALSClifford A. Stephens, Palo Alto, and Robert W.  
McCandless, Redwood, Calif.Original application Oct. 12, 1955, Ser. No. 540,104,  
now Patent No. 2,854,267, dated Sept. 30, 1958. Di-  
vided and this application Feb. 3, 1958, Ser. No.  
713,024

5 Claims. (Cl. 69—21)

This invention relates to a method for coating leather, especially leather shaft-sealing elements. This application is a division of our application Serial Number 540,104, filed October 12, 1955, which has become Patent No. 2,854,267, which was a continuation-in-part of our application Serial Number 519,862, filed July 5, 1955, now abandoned.

Leather has long been favored as far superior to most materials as a pliant sealing element for shafts, reciprocating rods and the like. Despite this, it is recognized that leather has certain disadvantages and fails to exhibit, to the degree desired, all the characteristics needed to meet the ever increasing requirements for a satisfactory seal. For example, leather varies widely in density, resilience, porosity and flexibility, all of which affect performance and suitability for use as sealing elements. Accordingly, over the years much effort has been directed toward improved processing procedures in an endeavor to provide a product of more uniform properties and longer service life. In addition, these attempts have included the augmentation of existing properties as well as the inclusion of new ones.

Another facet of the problem derives from the fact that certain desired properties of leather are customarily found only in combination with undesirable ones. For example, a leather having the desired flexibility is too soft to maintain good sealing contact with an eccentrically rotating shaft, or one which vibrates or whips as it rotates. Also, a flexible leather usually is quite porous. In consequence, it has a high reservoir capacity for lubricant—an advantageous quality. But this porosity is also attended by seepage of lubricant through the side walls of the leather—a highly undesirable quality. Previous efforts to seal the pores have destroyed the leather's capacity for storing lubricant and have stiffened the leather objectionably.

The primary object of the present invention is the provision of specially processed leather in which the desirable properties of leather are retained and augmented while other new properties are added.

Another object is the provision of a sealing element having a main body of leather with a coating bonded to at least one surface and serving to seal that surface against loss of lubricant by seepage to reduce greatly the surface friction, to increase the wearing qualities, and to add to the mechanical strength of the leather but changing its stiffness only to a minimum degree.

Yet another important object is the provision of a shaft seal leather sealing element specially treated on its shaft-contacting surface with a low-friction coating resistant to attack by lubricants and having long wearing qualities, whereby the torque loss caused by the seal is reduced to a minimum and the service life is increased.

## 2

A further object is the provision of a technique for coating leather with a veneer of elastomer applied as a liquid and allowed to dry before the application of heat and pressure vulcanize the coating to the surface area of the leather.

Still another object is a mode of vulcanizing and molding a ring area only of a plaque of leather whereby the unvulcanized center may be trimmed away and subsequently vulcanized and molded in a different size and shape.

Numerous other objects and advantages of the invention will become readily apparent from the following detailed specification taken in connection with the accompanying drawings illustrating typical modes of practicing the invention, and wherein:

Figure 1 is a sectional view through a shaft seal in its installed position and featuring a leather sealing member provided with a low-friction protective veneer on its outer surface only.

Figure 2 is a fragmentary enlarged view through a similar seal but having a protective veneer on both of its surfaces.

Figure 3 is a fragmentary sectional view on a further enlarged scale, taken through the sealing member of Figure 2 and showing the thickness of the coatings on an exaggerated scale for illustrative purposes only.

Figure 4 is a sectional view through a mold used in molding the leather and vulcanizing the elastomeric surface veneer.

Figure 5 is a fragmentary view of the mold on an enlarged scale showing the mold closed against a plaque of leather.

Figure 6 is an isometric view, partly in section, of the leather as it appears after removal from the mold.

Referring to Figure 1, it will be seen that our uniquely coated leather sealing element may be used in a shaft seal of any suitable construction, such as the seal generally designated 10. The radial flange 11 of our specially prepared leather sealing element is clamped between a metal washer 12 and the radial flange of a cupped outer case 13, by means of a cup-shaped inner case 14. Thus, the in-turned edge 15 of the casing 14 is held pressed against the washer 12 by the curled-in rim 16 of the outer case 13. The exterior cylindrical surface 17 of the outer case is accurately finished so as to have a snug press-fit with the side wall of a mounting bore 18 of a shaft housing 19. Seated against the shouldered inner end 20 of the bore 18 is a suitable bearing, such as an anti-friction bearing indicated at 21. This bearing may be held seated in the bore, as by a split spring keeper ring 22, which seats in a groove formed in the bore wall. The bearing 21 serves to support a shaft 23 centrally of the mounting bore 16.

The flexible sealing member interposed between the shaft 23 and the seal casing is formed principally of leather and is molded to provide an outer, radially extending, mounting flange 11 and a frusto-conical, axially extending, lip flange 24. This general shape and form of leather sealing lip is conventional and has been in common use for many years. The smallest diameter portion of its inner edge 25 may be held in sealing contact with the shaft 23 by a garter spring 26.

One of the unique features of the sealing element is the provision of a thin film or veneer 27 of a special elastomer bonded to the inner or shaft-contacting surface of the seal. If only one surface of the sealing member is to be coated, it is preferable to coat the hair side

rather than the opposite flesh side and to so mount the seal in the housing bore 18 that the elastomeric veneer is in contact with the shaft and is remote from the interior of the housing. The reasons for this will become apparent presently.

The principal functional ingredients of the veneer are a synthetic oil-resistant elastomer such as neoprene, a polyacrylic, a nitrile, or a chlorosulfonated polyethylene rubber having a suitable dry lubricant dispersed therein, such as graphite, molybdenum disulfide, mica or talc. These substances, compounded along with a suitable solvent vehicle in a manner to be disclosed below, are applied in liquid form to the surface of the leather sealing member and then vulcanized.

The elastomer does not penetrate beyond the base of the hair pore openings or of the surface crevices and other imperfections of the leather. This confinement of the veneer to the immediate surface area of the leather and its absence from the many voids in the body of the leather is highly important and has several advantages. Thus, the absence of elastomer from the interior body of the leather permits of a free and natural capillary flow of lubricant within the leather in a path generally parallel to the inner and outer surfaces. Secondly, the many voids naturally present in the leather are available as lubricant storage reservoirs. And, thirdly, the inherent flexibility of the body of the leather is not adversely affected by the presence of incompressible particles filling the voids. And, of special significance, the exterior surface of the leather or the one in contact with the rotating shaft 23 is sealed by a thin film of resilient material which is highly resistant to attack by lubricants, relatively impervious to both liquids and gases, and has a coefficient of friction at least 50% lower than the identical leather sealing element without the surface coating of this invention.

A second embodiment of the invention is illustrated in Figure 2 and differs from the Figure 1 design in that both sides of the leather sealing element have a surface veneer of elastomer. The same reference characters have been used as in the first form but are distinguishable by the use of a prime. The inner or flesh side of the sealing element is shown coated with a film of elastomer 28 corresponding to the coating 27 on the outer or hair side. The film thicknesses are somewhat exaggerated in the drawing since, in practice, a film thickness of 2 to 5 mils has been found most effective. Greater thicknesses can be employed but have a tendency to stiffen the leather objectionably and are not found to add to the service life of the sealing element to any material extent.

Coating both sides of the sealing element has certain advantages. It stiffens each side of the leather in equal degree; it provides a smooth finished surface on both sides of the sealing element; and it provides a substantially sealed reservoir for lubricant within the body of leather proper. The outer rim of this reservoir is sealed by the surrounding housing for the sealing element, leaving only the inner peripheral edge exposed to the interior of the appliance housing and the supply of oil therein. If the seal is to be used in a location not exposed to lubricating mediums, then the sealing element can be saturated with lubricant before installation. Thus, in either mode of use, the sealing edge of the lip has a continuous supply of oil available at all times. As soon as a film of oil between the shaft and the contacting edge of the seal tends to disappear, it is immediately replenished from the supply stored by capillary action in the body of the seal. Furthermore, the low friction coating in direct contact with the shaft contains a dry lubricant locked within the coating. This dry lubricant supplements the liquid lubricant within the body of the sealing element.

The coating compositions which we have found to be so satisfactory for surface films or coatings 27, 27' and 28 are elastomers or rubber-like synthetics incorporating one or more dry lubricants that are dispersed therein to

impart lubricity and other related properties important to a properly functioning seal. For example, the coating elastomer may be neoprene GN, or neoprene GRT, standard elastomeric polymers of chloroprene commercially available from E. I. du Pont de Nemours & Co. One hundred parts of this material should be compounded for rapid curing and mixed with between 10 and 60 parts by volume of a filling agent having lubricating properties such as graphite, molybdenum disulfide, mica or talc. (For graphite, the range by weight is between 20 and 120 parts per 100 parts elastomer.) This mixture is dissolved in a suitable solvent to provide a low viscosity solution of 5-20% solids. If a lower solids content is employed, the film does not distribute uniformly to provide a reliably continuous veneer, while a solution of higher solids content is too viscous for satisfactory results. It will, of course, be understood by those skilled in the handling of elastomeric compositions that suitable curing agents, anti-oxidants and accelerators are required as usual.

Suitable solvents include a mixture of one or more aromatics (toluene, benzene, or xylene and homologues of them) with paraffin hydrocarbons (e.g., gasoline or kerosene) or ketones (acetone, methyl-ethyl-ketone, and other liquids of the group) or naphthas. Wide variations of quantities can be used, and which solvent mixture is selected will depend on factors such as evaporation rate desired, cost, toxicity, etc.

The following specific examples suffice to illustrate the relative proportions of constituents which have been found particularly suitable in actual practice:

#### EXAMPLE I

|    | Neoprene rubber                 | Parts by weight |
|----|---------------------------------|-----------------|
| 35 | Constituents:                   |                 |
|    | Neoprene (chloroprene polymers) | 100             |
|    | Magnesium oxide                 | 4               |
|    | Zinc oxide                      | 5               |
|    | Phenyl-alpha-naphthylamine      | 2               |
| 40 | 2-mercaptoimidazoline           | 1               |
|    | Graphite                        | 30              |
|    | Total solids                    | 142             |
| 45 | Methyl-ethyl ketone             | 1148            |
|    | Toluene                         | 130             |
|    | Total liquids                   | 1278            |
| 50 | Grand total                     | 1420            |

Another composition giving excellent results employs copolymers of butyl acrylate and acrylonitrile or ethyl acrylate and chloro-ethyl-vinyl ether in lieu of neoprene. Such a composition may be compounded as follows:

#### EXAMPLE II

|    | Polyacrylic elastomer                                                          | Parts by weight |
|----|--------------------------------------------------------------------------------|-----------------|
| 60 | Constituents:                                                                  |                 |
|    | Lactoprene BA-12.5 (an acrylonitrile (87.5%)-butyl acrylate (12.5%) copolymer) | 100             |
|    | Stearic acid                                                                   | 1               |
|    | Sulfur                                                                         | 1               |
| 65 | Triethylene tetramine                                                          | 4               |
|    | Graphite                                                                       | 80              |
|    | Total solids                                                                   | 186             |
| 70 | Methyl-ethyl-ketone                                                            | 1504            |
|    | Toluene                                                                        | 170             |
|    | Total liquids                                                                  | 1674            |
| 75 | Grand total                                                                    | 1860            |

A third composition makes use of nitrile elastomer instead of neoprene. The following is an example of

components by weight found in practice to give excellent results:

## EXAMPLE III

*Nitrile elastomer*

| Constituents:                 | Parts by weight |
|-------------------------------|-----------------|
| Nitrile elastomer             | 100             |
| Sulfur                        | 2               |
| Stearic acid                  | 2               |
| Zinc oxide                    | 5               |
| Phenyl-alpha-naphthylamine    | 2               |
| Tetramethyl thiuram disulfide | 0.5             |
| Graphite                      | 70              |
| Total solids                  | 181.5           |
| Methyl-ethyl-ketone           | 1470            |
| Toluene                       | 164             |
| Total liquids                 | 1634            |
| Grand total                   | 1815.5          |

Still another composition which we have found to provide an excellent adherent veneer for leather employs chlorosulphonated polyethylene as a principal elastomeric component. This coating composition is made from the following ingredients:

## EXAMPLE IV

*Chlorosulphonated polyethylene*

| Constituents:                                | Parts by weight |
|----------------------------------------------|-----------------|
| Chlorosulphonated polyethylene               | 100             |
| Wood rosin, hydrogenated                     | 5               |
| Polymer of aromatic hydrocarbon <sup>1</sup> | 70              |
| Polymer of trimethyl-dihydro-quinoline       | 2               |
| Litharge                                     | 40              |
| Mercaptobenzothiazole                        | 2               |
| Diphenylguanidine                            | 1               |
| Graphite                                     | 70              |
| Total solids                                 | 290             |
| Methyl-ethyl-ketone                          | 2350            |
| Toluene                                      | 260             |
| Total liquids                                | 2610            |
| Grand total                                  | 2900            |

<sup>1</sup> Kenflex B, Kenrich Corp.

In any of these four examples, mica, talc, and molybdenum disulfide may be substituted for graphite, in equal volume. Graphite is, however, preferred.

Any of the foregoing compositions may be applied to the leather by dipping, dripping, spraying or other common coating techniques. However, since the deposition of a layer of the desired thickness and uniformity requires contact with the liquid over an appreciable period of time, the dipping and dripping-spraying techniques are particularly advantageous. Dipping is only practical when it is desired to coat both surfaces of the leather, while spraying may be used to coat either one or both surfaces.

The dipping process may be carried out by immersing the leather into a tank of the composition while the latter is agitated to keep the solid constituents in suspension. Immersion should be continued for a period of 10 to 60 minutes depending upon the thickness of coating desired. The leather is then removed and allowed to drain and dry at room temperature for a period of 6 to 24 hours after which it is ready for curing and molding to the desired shape.

The spray coating and dripping procedures will be obvious from the foregoing discussion of the dipping method. A spray, stream, or dripping of the coating liquid is applied to the leather for a period of 10 to 60 minutes. Care is, of course, exercised to distribute the coating composition evenly. If a coating is desired to only one surface, the spray or stream is directed in such a manner as to exclude it from one side, and it may be dripped only on the upper surface. A preferred method is to carry a series of leather blanks or plaques along a

conveyer, floating them on a film of the coating composition and passing them below a series of dripping stations, each of which may comprise a horizontal bar upon which the coating composition is being sprayed, so that it drips over the edges onto the blanks passing below. During the period of exposure, the flow of composition is discontinued and the pieces are allowed to dry preparatory to curing and molding which may be carried out by the aid of a mold of the type illustrated in Figures 4 and 6.

Figure 4 shows a 2-part mold closed against a plaque 40 of coated leather. The mold includes a lower female member 41 secured to a heated platen 42 of a molding press by means of a cap screw 43. The cooperating male mold member 44 is similarly secured to an upper platen 10 45 by a cap screw 46. It will be observed that each of the mold members has a large area cavity 47, 47 which does not contact the central portion 48 of the leather plaque. The outer opposed surface areas of the mold members 41 and 44 have supplemental surfaces uniformly spaced from one another and shaped to form a sealing element of L-shape in section as clearly indicated in the several figures of the drawing.

The narrow radial surfaces 49 and 50 of the mold members grip the center part of the plaque 40 firmly 25 and depress it into the general cup-shaped form shown in Figures 4 and 6 and hold it in this shape while the leather takes a permanent set and the elastomeric surface coatings are being vulcanized. The mold is closed under sufficient pressure to compress the leather from 20-30% 30 and so held for one minute while the molds are maintained at a temperature of approximately 275° F. It will, of course, be appreciated that the pressure, molding period and temperature may be varied over a considerable range as found to give the best results for the particular leather and coating composition being used. Molding may be carried out for longer periods (up to 90 seconds) at lower temperatures, and shorter periods (down to 10 seconds) at high temperatures, but temperatures higher than 325° F. should be avoided, else damage to the leather may result.

Slight curing of the coating opposite the cavities 47, 47 of the mold members may occur from the limited amount of heat reaching this area of the coating composition. The mold is held closed for such a short interval 45 that any curing which takes place will not interfere with the subsequent molding of a smaller size sealing element from the discarded central portion of the plaque 40. This will be best understood by the reference to Figure 6 showing the plaque 40 after it has been removed from the mold. The next step is to trim out the ring of leather desired for the sealing member. This is accomplished by placing the seal in a trimming lathe and cutting away the unvulcanized center along the conical surface indicated by a dotted line 50. The outer rim is likewise 55 trimmed at an angle such as that indicated by a dotted line 51. The narrow flanged ring so produced forms the sealing element of the completed seal.

The salvaged central portion 48 of the disc may be used to form radial-washer type seals or another cup-shaped sealing element of the same general shape shown in Figure 2 but of smaller diameter. Hence, it will be self-evident that this molding technique avoids waste and permits maximum usage of a given plaque of leather.

We claim:

65 1. That improvement in the treatment of leather for use as the flexible sealing member in a shaft seal which comprises, exposing one side of a plaque of tanned leather to contact with a liquid mixture of a heat curable flexible elastomeric material and a dry lubricant in a confined space until a coating of the mixture to the desired thickness adheres to the leather, drying the coating, forming a flanged cup from said plaque, subjecting the coating on the side wall and flanged rim of said cup to pressure and to heat not substantially in excess of 325° F. until said elastomeric material is cured, and cutting away the bot-

tom of said cup to provide a flanged ring having a long-wearing low-friction flexible oil barrier coating adhering to the surface on one side thereof.

2. An improvement in the manufacture of shaft seals of the type having a heat-molded leather sealing ring encased in a rigid mounting case and adapted to be pressed into a mounting bore surrounding a shaft; said improvement comprising the steps of coating the side surface of said leather intended to face outwardly with a dry lubricant dispersed in oil-resistant flexible elastomer, and vulcanizing said coating to the surface area only of said leather while simultaneously compressing the leather approximately 20% to 30% and while retaining it at a temperature not materially in excess of 325° F.

3. That improvement in the manufacture of shaft seals of the type having a heat-molded leather sealing ring encased in a rigid mounting case adapted to be pressed into a mounting bore surrounding a rotating shaft and comprising a leather ring having a radial flange and a flaring axial flange joined to one rim edge thereof, the free rim edge of said flaring flange being adapted to have light pressure running contact with the surface to be sealed against leakage of lubricant; said improvement comprising the steps of coating the surface of said leather intended for sealing contact before said leather is formed with said radial and axial flanges with a fluent mixture consisting of an oil-resistant flexible elastomer and graphite; and curing the coating for between about 10 and 90 seconds at a temperature not substantially in excess of 325° F. while holding said leather deformed to provide the radial and axial flanges and while holding it compressed to an extent less than one-half its natural state.

4. That improvement in the manufacture of annular molded leather rings which comprises coating at least one side of sheet leather with a layer of flexible elastomer dispersed in a solvent, drying the leather by exposure to

air, molding a ring-shaped area only of the coated sheet to a desired shape under pressure and a temperature not substantially in excess of 325° F. to vulcanize that portion of said coating under pressure, and trimming the molded and vulcanized portion of said ring from the unmolded and unvulcanized portion thereof.

5. That improvement in the manufacture of annular leather sealing rings for use in a shaft type seal which comprises coating the hair side of a sheet of leather with a liquid solution of uncured flexible elastomer, drying said coated sheet of leather, compressing and deforming a ring area of said coated sheet 20-30% while leaving the remainder of the sheet free of pressure, vulcanizing the elastomer in said ring area by heat, and trimming away the unvulcanized portions of the coated leather to either side of the vulcanized portion to provide an annular shaft sealing element having a thin resilient veneer of elastomer bonded to the hair side thereof.

References Cited in the file of this patent

UNITED STATES PATENTS

|           |                |               |
|-----------|----------------|---------------|
| 564,564   | Latulip        | July 21, 1896 |
| 1,054,265 | Baekeland      | Feb. 25, 1913 |
| 1,443,311 | Cook           | Jan. 23, 1923 |
| 1,472,744 | Butler         | Oct. 30, 1923 |
| 1,827,610 | Quimby         | Oct. 13, 1931 |
| 2,332,196 | Bjorksten      | Oct. 19, 1943 |
| 2,416,295 | Ehle           | Feb. 25, 1947 |
| 2,683,130 | D'Alelio       | July 6, 1954  |
| 2,700,623 | Hall           | Jan. 25, 1955 |
| 2,706,722 | Caldwell       | Apr. 19, 1955 |
| 2,715,617 | White          | Aug. 16, 1955 |
| 2,726,223 | Talet          | Dec. 6, 1955  |
| 2,836,972 | Cranker et al. | June 3, 1958  |